

# United States Patent [19]

Mohr

[11] Patent Number: 4,600,482

[45] Date of Patent: Jul. 15, 1986

[54] PROCESS FOR THE ELECTROCHEMICAL ROUGHENING OF ALUMINUM FOR USE AS PRINTING PLATE SUPPORTS, IN AN AQUEOUS MIXED ELECTROLYTE

[75] Inventor: Dieter Mohr, Schlangenbad, Fed. Rep. of Germany

[73] Assignee: Hoechst Aktiengesellschaft, Frankfurt am Main, Fed. Rep. of Germany

[21] Appl. No.: 726,242

[22] Filed: Apr. 23, 1985

## [30] Foreign Application Priority Data

Apr. 25, 1984 [DE] Fed. Rep. of Germany ..... 3415338

[51] Int. Cl.<sup>4</sup> ..... C25F 3/04

[52] U.S. Cl. ..... 204/129.4; 204/129.85;  
204/129.95

[58] Field of Search ..... 204/129.4, 129.85, 129.95

## [56] References Cited

### U.S. PATENT DOCUMENTS

- |           |         |                  |       |            |
|-----------|---------|------------------|-------|------------|
| 3,755,116 | 8/1973  | Terai et al.     | ..... | 204/129.95 |
| 3,887,447 | 6/1975  | Sheasby et al.   | ..... | 204/129.4  |
| 3,899,400 | 8/1975  | Patrie, et al.   | ..... | 204/33     |
| 4,052,275 | 10/1977 | Gumbinner et al. | ..... | 204/129.95 |
| 4,172,772 | 10/1979 | Ould et al.      | ..... | 204/129.85 |
| 4,339,315 | 7/1982  | Kikuchi et al.   | ..... | 204/129.85 |
| 4,367,124 | 1/1983  | Kikuchi et al.   | ..... | 204/17     |

## FOREIGN PATENT DOCUMENTS

- |         |        |                      |       |            |
|---------|--------|----------------------|-------|------------|
| 1400918 | 7/1975 | United Kingdom       | ..... | 204/129.75 |
| 2433491 | 1/1975 | Fed. Rep. of Germany | ..... | 204/129.95 |
| 1006207 | 9/1965 | United Kingdom       | ..... | 204/129.95 |

## OTHER PUBLICATIONS

A. J. Dowell, "The Alternating Current Etching of Aluminium Lithographic Sheet", Transactions of the Institute of Metal Finishing, vol. 57, pp. 138-144, 1979.

Primary Examiner—T. M. Tufariello  
Attorney, Agent, or Firm—Schwartz, Jeffery, Schwaab, Mack, Blumenthal & Evans

## [57] ABSTRACT

Disclosed is a process for electrochemically roughening aluminum or aluminum alloys for use as printing plate supports, in an aqueous mixed electrolyte solution containing hydrochloric acid (HCl) and, as an additional component, at least one haloalkanoic acid of the general formula  $\text{Hal}_x\text{H}_{y-x}\text{C}_z\text{—COOH}$ , in which Hal stands for a halogen atom, z is an integer from 1 to 5,  $y=2z+1$  and x is an integer from 1 to y. In particular, the solution contains from 0.5 to 10% by weight of HCl and from 0.1 to 8.0% by weight of haloalkanoic acid, for example, monochloroacetic acid or trifluoroacetic acid. The support materials which are particularly uniformly roughened are employed in the production of offset-printing plates.

15 Claims, No Drawings

PROCESS FOR THE ELECTROCHEMICAL  
ROUGHENING OF ALUMINUM FOR USE AS  
PRINTING PLATE SUPPORTS, IN AN AQUEOUS  
MIXED ELECTROLYTE

BACKGROUND OF THE INVENTION

The present invention relates to a process for the electrochemical roughening of aluminum which can be used for printing plate supports, said process being performed by means of alternating current in an aqueous mixed electrolyte.

Printing plates (this term referring to offset-printing plates, within the scope of the present invention) usually comprise a support and at least one radiation-sensitive (photosensitive) reproduction layer arranged thereon, the layer being applied to the support either by the user (in the case of plates which are not pre-coated) or by the industrial manufacturer (in the case of pre-coated plates). As a layer support material, aluminum or alloys thereof have gained general acceptance in the field of printing plates. In principle, it is possible to use these supports without modifying pretreatment, but they are generally modified in or on their surfaces, for example, by a mechanical, chemical and/or electrochemical roughening process (sometimes also called graining or etching in the literature), a chemical or electrochemical oxidation process and/or a treatment with hydrophilizing agents. In modern continuously working high-speed equipment employed by the manufacturers of printing plate supports and/or pre-coated printing plates, a combination of the aforementioned modifying methods is frequently used, particularly a combination of electrochemical roughening and anodic oxidation, optionally followed by a hydrophilizing step. Roughening is, for example, carried out in aqueous acids, such as aqueous solutions of HCl or HNO<sub>3</sub> or in aqueous salt solutions, such as aqueous solutions of NaCl or Al(NO<sub>3</sub>)<sub>3</sub>, or also in combinations of these components, using alternating current. The peak-to-valley heights (specified, for example, as mean peak-to-valley heights R<sub>z</sub>) of the roughened surface, which can thus be obtained, are in the range from about 1 to 15  $\mu\text{m}$ , particularly in the range from 2 to 8  $\mu\text{m}$ . The peak-to-valley height is determined according to DIN 4768, in the October 1970 version. The peak-to-valley height R<sub>z</sub> is then the arithmetic mean calculated from the individual peak-to-valley height values of five mutually adjacent individual measurement lengths.

Roughening is, *inter alia*, carried out in order to improve the adhesion of the reproduction layer to the support and to improve the water/ink balance of the printing form which results from the printing plate upon irradiation (exposure) and development. By irradiating and developing (or decoating, in the case of electrophotographically working reproduction layers), the ink-receptive image areas and the water-retaining non-image areas (generally the bared support surface) in the subsequent printing operation, are produced on the printing plate and thus the actual printing form is obtained. The final topography of the aluminum surface to be roughened is influenced by various parameters, as is explained by way of example in the text which follows:

The paper "The Alternating Current Etching of Aluminum Lithographic Sheet", by A. J. Dowell, published in *Transactions of the Institute of Metal Finishing*, 1979, Vol. 57, pages 138 to 144, presents basic comments on the roughening of aluminum in aqueous solu-

tions of hydrochloric acid, based on variations of the following process parameters and an investigation of the corresponding effects: The electrolyte composition is changed during repeated use of the electrolyte, for example, in view of the H<sup>+</sup>(H<sub>3</sub>O<sup>+</sup>) ion concentration (measurable by means of the pH) and in view of the Al<sup>3+</sup> ion concentration, with influences on the surface topography being observed. Temperature variations between 16° C. and 90° C. do not show an influence causing changes until temperatures are about 50° C. or higher, the influence becoming apparent, for example, as a significant decrease in layer formation on the surface. Variations in roughening time between 2 and 25 minutes lead to an increasing metal dissolution with increasing duration of action. Variations in current density between 2 and 8 A/dm<sup>2</sup> result in higher roughness values with rising current density. If the acid concentration is varied in a range from 0.17 to 3.3% of HCl, only negligible changes in pit structure occur between 0.5 and 2% of HCl. Below 0.5% of HCl, the surface is only locally attacked and at the high values, an irregular dissolution of Al takes place. An addition of SO<sub>4</sub><sup>2-</sup> ions or Cl<sup>-</sup> ions in the form of salts (e.g., by adding Al<sub>2</sub>(SO<sub>4</sub>)<sub>3</sub> or NaCl) can also influence the topography of the roughened aluminum. Rectification of the alternating current shows that, obviously, both half-wave types are necessary to obtain a uniform roughening.

Thus, it can be assumed that the use of aqueous HCl solutions as electrolyte solutions for the electrochemical roughening of support materials made of aluminum is principally known. With these solutions it is possible—as is also evidenced by a great number of commercially available printing plates—to achieve a uniform graining, which is particularly suitable for applications in the field of lithography, the roughness values of which vary within a range which in general is appropriate for practical use. For certain applications of printing plates (for example, in the case of certain negative-working reproduction layers) there is, however, required a uniform surface topography showing relatively little depth of roughening, which is difficult to obtain in the known electrolyte solutions on a basis of aqueous HCl solutions using modern, high-speed apparatus. For example, the process parameters must be kept within very narrow limits, which involves a process that can be controlled with great difficulty only.

The influence of the electrolyte composition on the quality of roughening is, for example, also described in the following publications, in which aqueous mixed electrolytes are employed:

German Offenlegungsschrift No. 22 50 275 (equivalent to British Published Application No. 1,400,918) specifies aqueous solutions containing from 1.0 to 1.5% of HNO<sub>3</sub> or from 0.4 to 0.6% of HCl and, optionally, from 0.4 to 0.6% of H<sub>3</sub>PO<sub>4</sub>, for use as electrolyte solutions in the roughening of aluminum for printing plate supports, by means of alternating current;

U.S. Pat. No. 3,887,447 specifies aqueous solutions containing from 0.2 to 2% of HCl and from 0.15 to 1.5% of H<sub>3</sub>PO<sub>4</sub>, for use as electrolyte solutions in the roughening of aluminum by means of alternating current;

U.S. Pat. No. 4,052,275 specifies aqueous solutions containing from 0.75 to 3.5% of HCl and from 0.2 to 1% of tartaric acid [2,3-dihydroxybutanedioic acid 1,4)] for use as electrolyte solutions in the roughening of aluminum;

U.S. Pat. No. 4,172,772 specifies aqueous solutions containing from 0.2 to 1.7% of HCl and from 0.5 to 4% of an alkanoic acid from C<sub>1</sub> to C<sub>4</sub> (particularly acetic acid, also known as ethanoic acid), for use as electrolyte solutions in the roughening of aluminum, by means of alternating current;

U.S. Pat. No. 4,367,124 specifies aqueous solutions containing from 0.35 to 3.5% of HCl and from 0.001 to 2% of a  $\beta$ -dicarbonyl compound, such as acetylacetone or acetoacetic acid ethyl ester, for use as electrolyte solutions in the roughening of aluminum support materials for printing plates;

U.S. Pat. No. 4,339,315 specifies aqueous solutions containing from 0.1 to 1.0 mole/l of HCl and from 0.01 to 1 mole/l of citric acid or malic acid [3-hydroxy-pentanetrioc acid (1,3,5) and 2-hydroxybutanedioic acid (1,4)], for use as electrolyte solutions in the roughening of aluminum support materials for printing plates; and

U.S. Pat. No. 3,755,116 specifies as addition of anti-corrosive agents—including monoamines, diamines, aliphatic aldehydes, carboxylic acid amides, such as acetamide, urea, chromic acid and non-ionic surfactants, such as polyethylene glycol ethers or esters—to an aqueous HCl electrolyte, for roughening aluminum for printing plate supports.

The known organic additives to aqueous acid electrolytes, such as HCl or HNO<sub>3</sub> solutions, have the disadvantage that in the case of high current loads (voltages) they become electrochemically unstable in modern continuously working web processing apparatus and decompose at least partially. The known inorganic additives, such as phosphoric acid, chromic or boric acid exhibit the disadvantage that quite often there is a local breakdown of their intended protective effect, as a consequence whereof single, particularly deep pits are formed at the respective spots.

In general, the known complex-forming additives accelerate the dissolution of the aluminum due to their "trapping" of released Al<sup>3+</sup> ions and thus cause an increased roughening action. As a result thereof, quite often no creation of new pores is initiated, but pores which are already existent continue to grow, i.e., increased pitting occurs. It is true that usually the growth of individual pores is stopped relatively soon by the known inhibiting additives, and the formation of new pores can be initiated. These inhibitors exhibit, however, the decisive disadvantage that this protective effect can collapse due to voids, alloying constituents, and the like, so that single pores which are too deep are obtained on a surface which otherwise shows a shallow and uniform roughening. Support materials exhibiting these kinds of defects are not suitable for lithographic purposes.

#### SUMMARY OF THE INVENTION

It is therefore an object of the present invention to provide a process for the electrochemical roughening of aluminum or aluminum alloys for printing plate supports. It is a further object of the invention to provide a process by which a uniformly roughened surface topography with a large range of variation in the mean peak-to-valley roughness values is achieved. It is still another object of the invention to provide a process in which long useful lives of the baths used can be obtained. It is yet another object of the invention to provide a composition for the electrochemical roughening of aluminum or aluminum alloys. It is still another object of the in-

vention to provide printing plate supports produced by the process of the invention.

These and other objects of the invention are achieved by a process for electrochemical roughening of a material selected from aluminum and aluminum alloys, comprising the steps of placing the material in an aqueous mixed electrolyte solution containing HCl and at least one haloalkanoic acid selected from Hal<sub>x</sub>H<sub>y-x</sub>C<sub>z</sub>—COOH, wherein Hal denotes a halogen atom, z is an integer from 1 to 5, y=2z+1, and x is an integer from 1 to y, and subjecting the material to the action of alternating current.

A composition for chemical roughening of aluminum or aluminum alloys comprises an aqueous mixed electrolyte solution containing HCl and at least one haloalkanoic acid selected from Hal<sub>x</sub>H<sub>y-x</sub>C<sub>z</sub>—COOH, wherein Hal denotes a halogen atom, z is an integer from 1 to 5, y=2z+1 and x is an integer from 1 to y.

A printing plate support material comprises a plate of aluminum or aluminum alloy having a roughened surface produced by placing the material in an aqueous mixed electrolyte solution containing HCl and at least one haloalkanoic acid selected from Hal<sub>x</sub>H<sub>y-x</sub>C<sub>z</sub>—COOH, wherein Hal denotes a halogen atom, z is an integer from 1 to 5, y=2z+1 and x is an integer from 1 to y and subjecting the material to the action of alternating current, and a radiation sensitive layer secured over the roughened surface.

#### DETAILED DESCRIPTION OF THE PREFERRED EMBODIMENTS

The invention is based on the known process for the electrochemical roughening of aluminum or aluminum alloys for use as printing plate supports in an aqueous mixed electrolyte solution containing HCl and at least one organic carboxylic acid, under the action of alternating current. In the process of the present invention, the organic carboxylic acid comprises a haloalkanoic acid corresponding to the general formula Hal<sub>x</sub>H<sub>y-x</sub>C<sub>z</sub>—COOH, in which Hal denotes a halogen atom, z is an integer from 1 to 5, y=2z+1 and x is an integer from 1 to y.

In a preferred embodiment, the aqueous electrolyte solution contains from 0.5 to 10.0% by weight, particularly from 0.8 to 5.0% by weight, of HCl and from 0.1 to 8.0% by weight, particularly from 0.2 to 5.0% by weight, of haloalkanoic acid(s).

The preferred acids corresponding to the general formula used in the process of the present invention include derivatives of acetic acid (ethanoic acid with z=1) and propionic acid (propanoic acid with z=2). It is, however, also possible to use derivatives of butyric acid (butanoic acid with z=3), valeric acid (pentanoic acid with z=4) and caproic acid (hexanoic acid with z=5). In the general formula, the index x preferably corresponds to an integer from 1 to 3 and among the halogens (fluorine, chlorine, bromine and iodine), F and Cl are preferred. Examples of compounds corresponding to the general formula include monochloroacetic acid, dichloroacetic acid and trichloroacetic acid (mono, di, and trichloroethanoic acid), monobromoacetic acid and tribromoacetic acid (mono and tribromomethanoic acid), trifluoroacetic acid (trifluoroethanoic acid),  $\alpha$ -chloropropionic acid (2-chloropropanoic acid),  $\beta$ -chloropropionic acid (3-chloropropanoic acid),  $\alpha$ -chlorocaproic acid [2-chloro-hexanoic acid (1)], monoiodoacetic acid (moniodo-ethanoic

acid), or  $\beta$ -chlorobutyric acid [3-chlorobutanoic acid (1)], in which  $x=1, 2$  or  $3$  and  $z=1, 2, 3$  or  $5$ .

Suitable base materials for the material to be roughened in accordance with this invention include aluminum or one of its alloys which, for example, have an Al content of more than 98.5% by weight and additionally contain small amounts of Si, Fe, Ti, Cu and Zn. Prior to the electrochemical treatment step, these aluminum support materials can be roughened—optionally after a precleaning step—by mechanical means (for example, by brushing and/or by treatment with an abrasive agent). All process steps can be carried out discontinuously using plates or foils, but preferably they are performed continuously using webs.

Particularly in continuous processes, the process parameters in the electrochemical roughening step are normally within the following ranges: temperature of the electrolyte 20° C. to 60° C., current density 3 to 200 A/dm<sup>2</sup>, dwell time of a material spot to be roughened in the electrolyte 1 to 300 seconds, and rate of flow of the electrolyte on the surface of the material to be roughened 5 to 100 cm/s. In discontinuous processes, the required current densities are rather in the lower region and the dwell times rather in the upper region of the ranges indicated in each case. A flow of the electrolyte can even be dispensed with in these processes. The type of current used usually is normal alternating current having a frequency of 50 to 60 Hz, but it is also possible to use modified current types, such as alternating current having different current intensity amplitudes for the anodic and for the cathodic current, lower frequencies, interruptions of current or superposition of two currents of different frequencies and wave shapes. The average peak-to-valley height  $R_z$  of the roughened surface is in a range from 1 to 15  $\mu$ m, in particular from 1.5 to 8.0  $\mu$ m. In addition to HCl and at least one of the halogenated carboxylic acids, the aqueous electrolyte may be admixed with aluminum ions in the form of aluminum salts, in particular 0.5 to 5.0% by weight of AlCl<sub>3</sub>.

Precleaning includes, for example, treatment with an aqueous NaOH solution with or without a degreasing agent and/or complex formers, trichloroethylene, acetone, methanol or other so-called aluminum pickles, which are commercially available. Following roughening or, in the case of several roughening steps, between the individual steps, it is possible to perform an additional etching treatment, during which in particular a maximum amount of 2 g/m<sup>2</sup> of material is removed (between the individual steps, up to 5 g/m<sup>2</sup>). Solutions which have an etching effect in general are aqueous alkali metal hydroxide solutions or aqueous solutions of salts having alkaline reactions or aqueous solutions of acids on a basis of HNO<sub>3</sub>, H<sub>2</sub>SO<sub>4</sub> or H<sub>3</sub>PO<sub>4</sub>, respectively. Apart from an etching treatment step performed between the roughening step and a subsequent anodizing step, non-electrochemical treatments are also known, which substantially have a purely rinsing and/or cleaning effect and are, for example, employed to remove deposits ("smut"), which have formed during roughening or simply to remove electrolyte remainders; dilute aqueous alkali metal hydroxide solutions or water can, for example, be used for these treatments.

The electrochemical roughening process according to the invention is preferably followed by an anodic oxidation of the aluminum in a further process step, in order to improve, for example, the abrasion and adhesion properties of the surface of the support material.

Conventional electrolytes, such as H<sub>2</sub>SO<sub>4</sub>, H<sub>3</sub>PO<sub>4</sub>, H<sub>2</sub>C<sub>2</sub>O<sub>4</sub>, amidosulfonic acid, sulfosuccinic acid, sulfosalicylic acid or mixtures thereof, may be used for the anodic oxidation. Particular preference is given to H<sub>2</sub>SO<sub>4</sub> and H<sub>3</sub>PO<sub>4</sub>, which may be used alone or in a mixture and/or in a multi-stage anodizing process.

The step of performing an anodic oxidation of the aluminum support material is optionally followed by one or more post-treating steps. Post-treating is particularly understood to be a hydrophilizing chemical or electrochemical treatment of the aluminum oxide layer, for example, an immersion treatment of the material in an aqueous solution of polyvinyl phosphonic acid according to German Pat. No. 16 21 478 (equivalent to British Published Application No. 1,230,447), an immersion treatment in an aqueous solution of an alkali metal silicate according to U.S. Pat. No. 3,181,461, or an electrochemical treatment (anodic oxidation) in an aqueous solution of an alkali metal silicate according to U.S. Pat. No. 3,902,976. These post-treatment steps serve, in particular, to improve even further the hydrophilic properties of the aluminum oxide layer, which are already sufficient for many fields of application, with the other well-known properties of the layer being at least maintained.

The materials prepared in accordance with this invention are used as supports for offset printing plates i.e., one or the two surfaces of the support material are coated with a radiation-sensitive composition, either by the manufacturers of presensitized printing plates or directly by the users. Suitable radiation- (photo-) sensitive layers basically include any layers which after irradiation (exposure), optionally followed by development and/or fixing, yield a surface in imagewise configuration which can be used for printing.

Apart from the silver halide-containing layers used for many applications, various other layers are known which are, for example, described in "Light-Sensitive Systems" by Jaromir Kosar, published by John Wiley & Sons, New York, 1965: colloid layers containing chromates and dichromates (Kosar, Chapter 2); layers containing unsaturated compounds, which, upon exposure, are isomerized, rearranged, cyclized, or crosslinked (Kosar, Chapter 4); layers containing compounds which can be photopolymerized, in which, on being exposed, monomers or prepolymers undergo polymerization, optionally with the aid of an initiator (Kosar, Chapter 5); and layers containing o-diazoquinones, such as naphthoquinone-diazides, p-diazoquinones, or condensation products of diazonium salts (Kosar, Chapter 7).

The layers which are suitable also include the electro-photographic layers, i.e., layers which contain an inorganic or organic photoconductor. In addition to the photosensitive substances, these layers can, of course, also contain other constituents, such as, for example, resins, dyes or plasticizers. In particular, the following photosensitive compositions or compounds can be employed in the coating of the support materials prepared in accordance with this invention:

Positive-working reproduction layers which contain o-quinone diazides, preferably o-naphthoquinone diazides, such as high or low molecular-weight naphthoquinone-1,2-diazide-2-sulfonic acid esters or amides as the light-sensitive compounds, which are described, for example, in German Pat. Nos. 854,890; 865,109; 879,203; 894,959; 938,233; 1,109,521; 1,144,705; 1,118,606; 1,120,273; 1,124,187 and 2,331,377 and in

European Patent Application Nos. 0,021,428 and 0,055,814;

negative-working reproduction layers which contain condensation products from aromatic diazonium salts and compounds with active carbonyl groups, preferably condensation products formed from diphenylaminediazonium salts and formaldehyde, which are described, for example, in German Pat. Nos. 596,731; 1,138,399; 1,138,400; 1,138,401; 1,142,871 and 1,154,123; U.S. Pat. Nos. 2,679,498 and 3,050,502 and British Published Application No. 712,606;

negative-working reproduction layers which contain co-condensation products of aromatic diazonium compounds, such as are, for example, described in German Pat. No. 20 65 732, which comprise products possessing at least one unit each of (a) an aromatic diazonium salt compound which is able to participate in a condensation reaction and (b) a compound which is able to participate in a condensation reaction, such as a phenol ether or an aromatic thioether, which are connected by a bivalent linking member derived from a carbonyl compound which is capable of participating in a condensation reaction, such as a methylene group;

positive-working layers according to German Offenlegungsschrift No. 26 10 842, German Pat. No. 27 18 254 or German Offenlegungsschrift No. 29 28 636, which contain a compound which, on being irradiated, splits off an acid, a monomeric or polymeric compound which possesses at least one C—O—C group which can be split off by acid (e.g., an orthocarboxylic acid ester group or a carboxylic acid amide acetal group), and, if appropriate, a binder;

negative-working layers, composed of photo-polymerizable monomers, photo-initiators, binders and, if appropriate, further additives. In these layers, for example, acrylic and methacrylic acid esters, or reaction products of diisocyanates with partial esters of polyhydric alcohols, are employed as monomers as described, for example, in U.S. Pat. No. 2,760,863 and No. 3,060,023, and in German Offenlegungsschriften Nos. 20 64 079 and 23 61 041;

negative-working layers according to German Offenlegungsschrift No. 30 36 077, which contain, as the photo-sensitive compound, a diazonium salt polycondensation product or an organic azido compound, and, as the binder, a high-molecular weight polymer with alkenylsulfonylurethane or cycloalkenylsulfonylurethane side groups.

It is also possible to apply photo-semiconducting layers to the support materials prepared in accordance with this invention, such as described, for example, in German Pat. Nos. 11 17 391; 15 22 497, 15 72 312, 23 22 046 and 23 22 047, as a result of which highly photosensitive electrophotographic printing plates are obtained.

From the coated offset printing plates prepared from the support materials produced in accordance with the present invention, the desired printing forms are obtained in known manner by imagewise exposure or irradiation, followed by washing out the non-image areas by means of a developer, for example, an aqueous alkaline developer solution.

The process according to this invention combines, *inter alia*, the following advantages:

The process products have a uniform surface topography, a property by which both the stability of print runs which can be achieved using printing forms produced from these support materials, and the water/ink balance during printing are positively influenced.

Compared with the use of electrolytes containing purely hydrochloric acid, "pitting" (pronounced depressions, as against the roughening of the surrounding surface) occurs less frequently and can even be suppressed completely.

Compared with the use of a non-halogenated carboxylic acid (see also comparative tests below), lower concentrations of halogenated carboxylic acid can be effective; the surface is more uniformly roughened and the amount of deposit formed is reduced.

These surface properties can be materialized without much equipment expenditure, and the properties can be achieved within a wide range of roughening intensities.

Employing this process, surfaces roughened in a particularly shallow and uniform manner can be achieved, which is not possible to the same degree using the known electrolytes.

The mixed electrolyte used in the process of this invention is electrochemically stable, i.e., it practically does not decompose when high current loads (voltages) are applied.

In the above description and in the Examples which follow, percentages denote percent by weight, unless otherwise stated. Parts by weight (p.b.w.) are related to parts by volume (p.b.v.) as grams are related to cm<sup>3</sup>.

#### EXAMPLES 1 TO 21 AND COMPARATIVE EXAMPLES C1 TO C17

An aluminum sheet was first treated with an aqueous solution containing 20 g/l of NaOH, at room temperature, for a time of 60 seconds and was then freed from any remaining alkaline residues by briefly dipping it into a solution of a composition corresponding to that of the roughening electrolyte. Roughening was performed in the electrolyte systems and under the conditions described in the Tables below. Roughening was followed by an anodic oxidation in an aqueous electrolyte with a content of H<sub>2</sub>SO<sub>4</sub> and Al<sup>3+</sup> ions, until a layer weight of 3 g/m<sup>2</sup> was reached.

Classifying into quality grades (surface topography) was made by visual assessment under a microscope, a homogeneously roughened surface which was free from pitting being assigned quality grade "1" (best grade). A surface with severe pitting of a size exceeding 100 µm or with an extremely non-uniformly roughened or almost "mill-finished" surface was assigned quality grade "10" (worst grade). Surfaces of qualities between these two extreme values were assigned quality grades "2" to "9". All examples and comparative examples were performed using symmetric alternating current of a frequency of 50 Hz, one electrode being constituted by the aluminum sheet and the other electrode being constituted by a graphite plate.

TABLE

| Example No. | Concentration and Composition of the aqueous electrolyte |                                        |                           | Current density (A/dm <sup>2</sup> ) | Roughening time (sec) | Peak-to-valley height R <sub>z</sub> (μm) | Quality grade |
|-------------|----------------------------------------------------------|----------------------------------------|---------------------------|--------------------------------------|-----------------------|-------------------------------------------|---------------|
|             | Quantity of HCl (%)                                      | Admix-ture                             | Quantity of admixture (%) |                                      |                       |                                           |               |
| C1          | 1.2                                                      | —                                      | —                         | 40                                   | 15                    | 4.29                                      | 4             |
| C2          | 1.2                                                      | —                                      | —                         | 60                                   | 10                    | 4.03                                      | 4             |
| C3          | 1.2                                                      | —                                      | —                         | 80                                   | 8                     | 4.97                                      | 5             |
| C4          | 1.2                                                      | —                                      | —                         | 100                                  | 6                     | 5.45                                      | 4             |
| C5          | 1.2                                                      | —                                      | —                         | 40                                   | 20                    | 5.14                                      | 4             |
| C6          | 1.2                                                      | —                                      | —                         | 80                                   | 10                    | 5.91                                      | 4             |
| C7          | 1.2                                                      | —                                      | —                         | 100                                  | 8                     | 6.76                                      | 5             |
| C8          | 1.2                                                      | —                                      | —                         | 120                                  | 6                     | 8.49                                      | 6             |
| C9          | 1.2                                                      | —                                      | —                         | 40                                   | 25                    | 6.21                                      | 4             |
| C10         | 1.2                                                      | —                                      | —                         | 80                                   | 12                    | 7.88                                      | 6             |
| C11         | 1.2                                                      | —                                      | —                         | 120                                  | 8                     | 8.03                                      | 7             |
| C12         | 1.2                                                      | —                                      | —                         | 40                                   | 38                    | 8.13                                      | 6             |
| C13         | 1.2                                                      | CH <sub>3</sub> COOH                   | 2.0                       | 80                                   | 8                     | 4.57                                      | 4             |
| C14         | 1.2                                                      | CH <sub>3</sub> COOH                   | 2.0                       | 100                                  | 10                    | 6.69                                      | 5             |
| C15         | 1.2                                                      | CH <sub>3</sub> COOH                   | 2.0                       | 60                                   | 10                    | 3.83                                      | 3             |
| C16         | 1.2                                                      | CH <sub>3</sub> COOH                   | 5.0                       | 80                                   | 8                     | 4.20                                      | 3             |
| C17         | 1.2                                                      | CH <sub>3</sub> COOH                   | 5.0                       | 100                                  | 10                    | 6.41                                      | 4             |
| 1           | 1.2                                                      | ClCH <sub>2</sub> COOH                 | 0.5                       | 60                                   | 10                    | 3.71                                      | 2             |
| 2           | 1.2                                                      | ClCH <sub>2</sub> COOH                 | 0.5                       | 80                                   | 10                    | 4.97                                      | 2             |
| 3           | 1.2                                                      | ClCH <sub>2</sub> COOH                 | 0.5                       | 100                                  | 10                    | 6.22                                      | 3             |
| 4           | 1.2                                                      | ClCH <sub>2</sub> COOH                 | 2.0                       | 80                                   | 8                     | 3.80                                      | 2             |
| 5           | 1.2                                                      | ClCH <sub>2</sub> COOH                 | 2.0                       | 100                                  | 10                    | 5.47                                      | 3             |
| 6           | 1.2                                                      | ClCH <sub>2</sub> COOH                 | 5.0                       | 100                                  | 10                    | 5.04                                      | 3             |
| 7           | 1.2                                                      | Cl <sub>2</sub> CHCOOH                 | 0.5                       | 80                                   | 10                    | 4.27                                      | 2             |
| 8           | 1.2                                                      | Cl <sub>2</sub> CHCOOH                 | 2.0                       | 100                                  | 10                    | 4.48                                      | 3             |
| 9           | 1.2                                                      | Cl <sub>2</sub> CHCOOH                 | 5.0                       | 60                                   | 18                    | 5.43                                      | 4             |
| 10          | 1.2                                                      | Cl <sub>3</sub> CCOOH                  | 0.5                       | 40                                   | 25                    | 4.18                                      | 2             |
| 11          | 1.2                                                      | Cl <sub>3</sub> CCOOH                  | 0.5                       | 60                                   | 10                    | 3.06                                      | 1             |
| 12          | 1.2                                                      | Cl <sub>3</sub> CCOOH                  | 0.5                       | 80                                   | 10                    | 3.45                                      | 1             |
| 13          | 1.2                                                      | Cl <sub>3</sub> CCOOH                  | 1.0                       | 100                                  | 10                    | 3.96                                      | 2             |
| 14          | 1.2                                                      | Cl <sub>3</sub> CCOOH                  | 2.0                       | 40                                   | 25                    | 3.96                                      | 1             |
| 15          | 1.2                                                      | BrCH <sub>2</sub> COOH                 | 2.0                       | 80                                   | 12                    | 3.90                                      | 2             |
| 16          | 1.2                                                      | Br <sub>3</sub> CCOOH                  | 2.0                       | 100                                  | 10                    | 4.23                                      | 3             |
| 17          | 1.2                                                      | F <sub>3</sub> CCOOH                   | 0.2                       | 60                                   | 10                    | 2.81                                      | 1             |
| 18          | 1.2                                                      | F <sub>3</sub> CCOOH                   | 0.5                       | 120                                  | 8                     | 4.23                                      | 1             |
| 19          | 1.2                                                      | CH <sub>3</sub> ClCHCOOH               | 2.0                       | 100                                  | 10                    | 5.49                                      | 3             |
| 20          | 1.2                                                      | ClCH <sub>2</sub> CH <sub>2</sub> COOH | 2.0                       | 100                                  | 10                    | 5.68                                      | 4             |
| 21          | 1.2                                                      | C <sub>4</sub> H <sub>9</sub> ClCHCOOH | 2.0                       | 80                                   | 12                    | 5.13                                      | 3             |

## EXAMPLE 22

An aluminum sheet prepared in accordance with Example 12 was immersed into an aqueous solution containing 5 g/l of polyvinylphosphonic acid, at a temperature of 40° C. and for a duration of 30 seconds; then it was rinsed with fully deionized water and dried. For obtaining a lithographic printing plate, the sheet was coated with the following negative-working photosensitive solution:

0.70 p.b.w. of the polycondensation product of 1 mole of 3-methoxy-diphenylamine-4-diazonium sulfate and 1 mole of 4,4'-bismethoxymethyl-diphenyl ether, precipitated as the mesitylene sulfonate,

3.40 p.b.w. of an 85% strength aqueous H<sub>3</sub>PO<sub>4</sub>,

3.00 p.b.w. of a modified epoxide resin, obtained by reacting 50 parts by weight of an epoxide resin having a molecular weight of less than 1,000 and 12.8 parts by weight of benzoic acid in ethylene glycol monomethyl ether, in the presence of benzyltrimethylammonium hydroxide,

0.44 p.b.w. of finely-ground Heliogen Blue G (C.I. 74,100),

62.00 p.b.v. of ethylene glycol monomethyl ether,

30.60 p.b.v. of tetrahydrofuran, and

8.00 p.b.v. of butyl acetate.

The printing plate was imagewise exposed and rapidly developed, without scum, with an aqueous solution containing Na<sub>2</sub>SO<sub>4</sub>, MgSO<sub>4</sub>, H<sub>3</sub>PO<sub>4</sub>, a non-ionic surfac-

tant, benzyl alcohol and n-propanol. When the printing form was used for printing, a very good ink-water balance and an excellent layer adhesion were stated.

## EXAMPLE 23

An aluminum foil, which had been prepared in accordance with Example 6 and post-treated in accordance with Example 22, was coated with the following positive-working photosensitive solution:

6.60 p.b.w. of a cresol/formaldehyde novolak (softening range 105° to 120° C., according to DIN 53,181),

1.10 p.b.w. of the 4-(2-phenyl-prop-2-yl)phenyl ester of naphthoquinone-1,2-diazide-2-sulfonic acid-4,

0.60 p.b.w. of 2,2'-bis-(naphthoquinone-1,2-diazide-2-sulfonyloxy-5)-dinaphthyl-1,1'-methane,

0.24 p.b.w. of naphthoquinone-1,2-diazide-2-sulfonylchloride-4,

0.08 p.b.w. of crystal violet, and

91.36 p.b.w. of a mixture of 4 p.b.v. of ethylene glycol monomethyl ether, 5 p.b.v. of tetrahydrofuran and 1

60 p.b.v. of butyl acetate.

By imagewise exposure and development in an aqueous solution containing Na<sub>2</sub>SiO<sub>3</sub>, Na<sub>3</sub>PO<sub>4</sub> and NaH<sub>2</sub>PO<sub>4</sub>, a printing form was produced from this plate, which gave 140,000 prints.

## EXAMPLE 24

A support material prepared in accordance with Example 18 was coated with a solution of the following

composition in order to obtain an electrophotographic offset printing plate:

10.00 p.b.w. of 2-vinyl-5-(4'-diethylaminophenyl)-4-(2'-chlorophenyl)-oxazole,

10.00 p.b.w. of a copolymer of styrene and maleic anhydride, having a softening point of 210° C.,

0.02 p.b.w. of  $\textcircled{R}$ Rhodamine FB, and

300.00 p.b.w. of ethylene glycol monomethyl ether.

By means of a corona, the layer was negatively charged to about 400 V in the dark. The charged plate 10 was imagewise exposed in a reprographic camera and then developed with an electrophotographic suspension-type developer obtained by dispersing 3.0 p.b.w. of magnesium sulfate in a solution of 7.5 p.b.w. of pentaerythritol resin ester in 1,200 p.b.v. of an isoparaffin mixture having a boiling range from 185° to 210° C. After removal of excess developer liquid, the developer was fixed and the plate was immersed, during 60 seconds, in a solution comprised of 35 p.b.w. of sodium metasilicate.9H<sub>2</sub>O, 140 p.b.w. of glycerol, 550 p.b.w. of 20 ethylene glycol and 140 p.b.w. of ethanol. Then, the plate was rinsed with a vigorous jet of water, whereby those areas of the photoconductor layer, which were not covered by toner, were removed. After rinsing, the printing form was ready for printing.

What is claimed is:

1. A process for the electrochemical roughening of a material selected from aluminum and aluminum alloys, comprising the steps of:

placing the material in an aqueous mixed electrolyte 30 solution containing HCl and at least one haloalkanoic acid selected from  $\text{Hal}_x\text{H}_{y-x}\text{C}_z\text{—COOH}$ , wherein Hal denotes a halogen atom, z is an integer from 1 to 5, y=2z+1, and x is an integer from 1 to y; and

subjecting the material to the action of alternating current.

2. A process as claimed in claim 1, wherein the mixed electrolyte contains from about 0.5 to about 10% by weight of HCl and from about 0.1 to about 8.0% by 40 weight of haloalkanoic acid.

3. A process as claimed in claim 1, wherein the mixed electrolyte contains from about 0.8 to about 5.0% by weight of HCl and from about 0.2 to about 5.0% by weight of haloalkanoic acid.

4. A process as claimed in claim 1, wherein z is 1 or 2, x is 1 to 3, and Hal is F or Cl.

5. A process as claimed in claim 1, wherein said process is continuous, and wherein the rate of flow of said electrolyte over the surface of said material is from 50 about 5 to about 100 cm/sec.

6. A process as claimed in claim 5, wherein said aqueous mixed electrolyte solution is at a temperature of from about 20° C. to about 60° C., the density of said alternating current is from about 3 to about 200 A/dm<sup>2</sup>, and the dwell time of said material in said solution is from about 1 to about 300 seconds.

7. A process as claimed in claim 1, wherein said process further includes a pretreatment step with an aqueous NaOH solution.

8. A process as claimed in claim 7, wherein said NaOH solution further contains one or more components selected from degreasing agents, complex formers, trichloroethylene, acetone and methanol.

9. A process as claimed in claim 1, wherein the roughening of the material surface is performed in 2 or more stages, and when an additional etching treatment is performed after each said roughening stage.

10. A composition for chemical roughening of aluminum or aluminum alloys, comprising:

an aqueous mixed electrolyte solution containing HCl and at least one haloalkanoic acid selected from  $\text{Hal}_x\text{H}_{y-x}\text{C}_z\text{—COOH}$ , wherein Hal denotes a halogen atom, z is an integer from 1 to 5, y=2z+1 and x is an integer from 1 to y.

11. A composition as claimed in claim 10, wherein said mixed electrolyte solution contains from about 0.5 to about 10% by weight HCl and from about 0.1 to about 8.0% by weight of the haloalkanoic acid.

12. A composition as claimed in claim 10, wherein said mixed electrolyte solution contains from about 0.8 to about 5.0% by weight HCl and from about 0.2 to about 5.0% by weight of haloalkanoic acid.

13. A composition as claimed in claim 10, wherein z is 1 or 2, x is 1 to 3 and Hal is F or Cl.

14. A printing plate support material, comprising:  
a plate of aluminum or aluminum alloy having a roughened surface produced by placing the material in an aqueous mixed electrolyte solution containing HCl and at least one haloalkanoic acid selected from  $\text{Hal}_x\text{H}_{y-x}\text{C}_z\text{—COOH}$ , wherein Hal denotes a halogen atom, z is an integer from 1 to 5, y=2z+1 and x is an integer from 1 to y, and subjecting the material to the action of alternating current; and

45 a radiation sensitive layer secured over said roughened surface.

15. A printing plate support material as claimed in claim 14, wherein the average peak-to-valley roughness of the roughened surface is in the range of from about 1 to about 15  $\mu\text{m}$ .

\* \* \* \* \*